

R. D. MERSHON,  
FORMING DIELECTRIC FILMS,  
APPLICATION FILED FEB. 18, 1920.

1,388,874.

Patented Aug. 30, 1921.



Ralph D. Mershon INVENTOR  
Kerr, Page, Cooper & Hayward BY ATTORNEYS

# UNITED STATES PATENT OFFICE.

RALPH D. MERSHON, OF NEW YORK, N. Y.

## FORMING DIELECTRIC FILMS.

1,388,874.

Specification of Letters Patent. Patented Aug. 30, 1921.

Application filed February 18, 1920. Serial No. 359,573.

To all whom it may concern:

Be it known that I, RALPH D. MERSHON, a citizen of the United States of America, residing at New York, in the county and State of New York, have invented certain new and useful Improvements in Forming Dielectric Films, of which the following is a full, clear, and exact description.

As is well known, the action of electrolytic condensers, rectifiers and other devices depends upon the film which may be formed upon the surface of aluminum, tantalum and other metals immersed in certain electrolyte and subjected to the electric current; which film possesses the remarkable property of allowing current to flow from the electrolyte to the electrode with but little or no opposition, but of strongly opposing current tending to flow from the electrode to the electrolyte. In tending to pass through the film the current exerts a stress thereon which may be conveniently termed "film stress." Flow of current from the electrolyte to the electrode is accompanied by the formation of minute holes or perforations for its passage, but when the direction of the current is reversed these holes will be healed up by re-formation of the film over them. The re-formation, however, is at the expense of the underlying metal, as is the original formation of the film, and hence repeated perforation and re-formation will in the course of time seriously corrode the metal and eventually destroy the electrode. Hence it is in general highly desirable to have the film stress constant in direction, that is, tending to send current from the electrode to the electrolyte, so that perforation will not occur. For this reason the practice heretofore in forming the films has been to use direct current for the purpose, the positive pole of a suitable source of such current being connected to the electrodes and the negative pole to the electrolyte. In subsequent use of the filmed electrodes in a condenser on an alternating current circuit reversal of the film stress is prevented by "exciting" the condenser, that is, by providing a unidirectional E. M. F. opposing that between the electrolyte and the electrodes, as fully explained in my prior Patent No. 1,077,628, dated November 13, 1913. In forming films with direct current the voltage employed is usually raised a little above the maximum voltage at which the apparatus is to be used

on alternating current and the formation preferably continued at this voltage until the current passed by the films has fallen to a suitably low value. It has been found that the behavior of the film is as if its thickness were a direct function of the forming voltage, that is, the higher the forming voltage the thicker the film. But it has also been found that there is a point, which may be conveniently termed the critical voltage, beyond which increase of the forming voltage does not materially increase the thickness of the film; or, if it does, it requires an indefinitely long time for its accomplishment.

I have discovered, however, that the films may be formed by the simultaneous use of both direct and alternating current, even with the apparatus in operation as a condenser during practically the entire period of formation, and it is accordingly the chief object of my present invention to provide a convenient and effective method for the purpose. To this and other ends the invention consists in the novel features hereinafter described.

The drawing illustrates diagrammatically the preferred method of carrying out my invention.

In carrying out the invention in the preferred manner the condenser is first excited at a low unidirectional voltage, thus forming or partially forming the film up to that voltage, and, while the direct voltage is still impressed, alternating voltage of low value is also supplied. The application of the alternating voltage causes an increase of current through the D. C. source of exciting current, depending upon the value of the alternating voltage employed, as will be readily understood. The addition of the alternating voltage correspondingly increases the film stress and hence produces further film formation and by thus increasing the resistance of the films reduces the direct current flowing. When the latter has fallen well below the permissible current capacity of the direct current machine supplying the direct current the alternating voltage is raised until the current through the D. C. machine has risen to the maximum value permissible for the machine. The increase of alternating voltage produces further film formation, with consequent decrease of direct current passed, and when the latter has again fallen to a suitably low value the alternating voltage

is again raised. This process is continued until the alternating voltage is the maximum that can be employed without reversing the film stress. When this point is 5 reached the unidirectional voltage is increased by a convenient amount, and when, because of further film formation, the direct current passed by the films has fallen sufficiently the alternating voltage is again increased. 10

The steps described are repeated as often as necessary to form the films up to the thickness desirable in subsequent operation of the condenser, or even farther. In fact, 15 if the condenser is intended to be operated on a voltage at or near the critical value of the film stress the formation may be carried on at voltages higher, even considerably higher, than the critical value.

20 Instead of increasing the forming voltages by steps as described, the progressive increase may be gradual, the unidirectional and alternating voltages being increased simultaneously and gradually but always at such 25 rates as will avoid the possibility of reversing the film stress.

The films may be formed in a cold electrolyte, or, if heat-resistant films are desired, the formation may be effected in a hot electrolyte, for example as described in my 30 prior patent No. 1,012,889, dated December 11, 1911.

My present invention possesses several 35 important advantages. In the first place, a much smaller direct current generator is required than where the formation is carried up to the maximum desired film stress by means of direct current alone, since in the latter case the generator must supply and 40 carry the current involved by the high voltage used. In the present method the direct current machine must also carry the forming current, but at a much lower voltage. Secondly, since the condenser is connected with 45 an alternating current circuit during formation of the films, it is possible at any stage to determine the power factor and other constants of the condenser merely by inserting the proper measuring or indicating 50 instruments in the circuit without disturbing the internal or external connections of the condenser.

In practising the invention in the preferred manner the electrodes which are to be 55 filmed are connected to the alternating source as a condenser, that is, half the plates are connected to one terminal of the source and the other half to the other terminal. Thus in the drawing, the plates 10, immersed 60 in a suitable electrolyte 11 contained in a tank 12, are connected to one terminal of the alternating source 14, through the medium of the autotransformer 15, and the other plates, 16, are similarly connected to the 65 other terminal. In each case the connection

of the plates to the autotransformer is variable, as indicated, so that the impressed voltage may be varied as desired. The positive pole of the unidirectional source 17 is connected through a variable resistance 18 to the neutral point of an autotransformer 19 which is itself connected across the alternating source, and the negative pole is connected to the electrolyte, as by means of a cathode 20, composed of gold, nickel, or other suitable non-filming material. In starting the formation of the film the variable connections are set to give the desired low voltages and are shifted to increase the voltages as already described. It is to be 70 understood that I do not limit myself to any particular method of varying the voltages. In order to prevent reversal of the film stress there is a minimum value of the unidirectional voltage at the plates, relative to the 75 alternating voltage, at or above which the former should be kept regardless of absolute values. This minimum value is one-half the maximum instantaneous value of the alternating voltage. Thus, in the case of an alternating E. M. F. wave of simple sine form, and representing the value of the alternating voltage by  $E$  (the square root of the mean of the squares of the instantaneous values), the unidirectional voltage should, 80 theoretically, never be less than  $\frac{1}{2}\sqrt{2}E$ , though it may be as much higher as desired.

It is to be understood that the invention is not limited to the exact procedure herein 85 specifically described but can be practised in other ways without departure from its 90 spirit.

I claim:

1. In the art of forming dielectric films of 105 the kind described, the improvement comprising impressing upon the electrodes immersed in a suitable electrolyte both direct and alternating voltages of such relative values as to prevent reversal of the film stress.

2. In the art of forming dielectric films of 110 the kind described, the improvement comprising impressing on the electrodes immersed in a suitable electrolyte both direct and alternating voltages of such relative values as to produce a film stress constantly 115 directed from the electrodes toward the electrolyte.

3. In the art of forming dielectric films of 120 the kind described, the improvement comprising immersing the electrodes in a suitable electrolyte, connecting the electrodes to a source of alternating voltage in the manner of a condenser and connecting the electrodes to the positive pole and the electrolyte to the negative pole of a source of unidirectional voltage to impress both unidirectional and alternating voltages of suitable values, and thereafter increasing the alternating and unidirectional voltages.

4. In the art of forming dielectric films 125

- of the kind described, the improvement comprising immersing the electrodes in a suitable electrolyte, impressing on the electrodes both unidirectional and alternating voltages of suitable values, and thereafter increasing the unidirectional and alternating voltages with such relative values as will prevent film stress from the electrolyte to the electrodes.
- 5 5. In the art of forming dielectric films of the kind described, the improvement comprising immersing the electrodes in a suitable electrolyte, impressing unidirectional voltage on the electrodes to partially form the films, and while supplying unidirectional voltage to the electrodes, operating the apparatus as a condenser in connection with a source of alternating voltage.
- 10 6. In the art of forming dielectric films of the kind described, the improvement comprising impressing on the electrodes immersed in a suitable electrolyte a unidirectional voltage of relatively low value to start formation of the films and exert a film stress from the electrodes to the electrolyte, and later impressing on the electrodes an alternating voltage of a value too low to reverse the film stress.
- 15 7. In the art of forming dielectric films of the kind described, the improvement comprising impressing on the electrodes immersed in a suitable electrolyte a unidirectional voltage of relatively low value to start formation of the films and exert a film stress from the electrodes to the electrolyte, impressing on the electrodes an alternating voltage of a value too low to reverse the film stress, and when the direct current through the unidirectional source
- 20 40 has decreased to a suitable value increasing the alternating voltage to increase the film stress from the electrodes to the electrolyte.
- 25 8. In the art of forming dielectric films of the kind described, the improvement comprising impressing on the electrodes immersed in a suitable electrolyte a unidirectional voltage of suitable value to start formation of the films and exert a film stress from the electrodes to the electrolyte, impressing on the electrodes an alternating
- 30 35 45 50 voltage of a value high enough to increase the film stress without reversal thereof and without materially exceeding the permissible current-carrying capacity of the source of unidirectional voltage, increasing the alternating voltage one or more times without reversing the film stress, increasing the unidirectional voltage to a safe value, and repeating one or more of the foregoing steps until the films are formed to the thickness 60 65 70 75 80 85 90 95 desired.
9. In the art of forming dielectric films of the kind described, the improvement comprising impressing on the electrodes immersed in a suitable electrolyte a unidirectional voltage of relatively low value and thereby forming the films up to such voltage, impressing a relatively low alternating voltage on the electrodes until the resulting increased current through the films has fallen to a suitable value, and thereafter increasing the alternating and unidirectional voltages without causing flow of current from the electrolyte to the electrodes and without materially exceeding the current-carrying capacity of the source of unidirectional voltage.
10. In the art of forming dielectric films of the kind described, the improvement comprising subjecting the electrodes immersed in a suitable electrolyte to unidirectional and alternating voltages, and progressively increasing such voltages without causing a film stress from the electrolyte to the electrodes and without materially exceeding the permissible current-carrying capacity of the source of unidirectional voltage, until the films are formed up to, at least the maximum voltage at which the electrodes are to be used in an electrolytic condenser.
11. In the art of forming dielectric films of the kind described, the improvement comprising impressing on the electrodes immersed in a suitable electrolyte both unidirectional and alternating voltages, and progressively increasing such voltages at suitable rates until the critical film stress is exceeded.

In testimony whereof I hereunto affix my signature.

RALPH D. MERSHON.